

## UNITED STATES PATENT OFFICE

2,127,252

## TEXTILE TREATMENT

August C. Fischer, St. Louis County, Mo.

No Drawing. Application August 10, 1936,  
Serial No. 95,176

5 Claims. (CL. 21—5)

This invention relates to improvements in textile treatment, and more particularly to improved materials and processes for the treatment of animal fibers and textiles, such as wool, against damage by insect life, the usual example of which is the moth larvae.

The present invention constitutes a continuation in part of the subject matter disclosed and claimed in my copending application filed May 4, 10 1935, and bearing Serial No. 19,777.

Numerous processes and materials have been heretofore proposed and used, with indifferent success, for the protection of wool and other animal fibers and textiles against the ravages of moth. Probably the least unsatisfactory form of treatment involves an immersion of the fabric in a bath of a treating liquid carrying an insectifuge. Due to the fact that by far the greater proportion of garments to be treated against moth attack consist of wool and woolen fabrics and textiles, and since as is known, only a limited quantity of water may be employed in or on woolen fabrics without undesirable or harmful effects, the mothproofing materials heretofore utilized have been largely composed of chemicals appreciably soluble in liquid hydrocarbons, and for this reason, organic materials have been usually employed in order to obtain the requisite solubility. These materials, considered as a class, exhibit the extreme disadvantage of being too high in cost for general, frequent and repeated usage, the economic factor having heretofore been the chief deterrent to their widespread and general adoption.

Certain inorganic chemicals have heretofore been proposed for use in mothproofing fabrics. The inorganic chemicals having the requisite toxic and moth repellent effect are however subject to the disadvantages of being either prohibitive in cost for widespread and general use, or of being of such low or negligible solubility in liquid hydrocarbons as to prevent their application in this manner, and of such low solubility in aqueous solution as to require an amount of water harmful to the fabric, in order to effect a uniform distribution of the toxic or repellent through the wool. The present invention has as its general and major objective, the attainment of a mothproofing process which may be practiced at extremely low cost, is susceptible of easy and widespread commercial application, may be practiced by anyone without special training or skill, and which overcomes all of the above noted disadvantages attending the processes attempted

for the same purpose, prior to the developments of the applicant in this field.

A further object of the invention is attained in a treatment for mothproofing, involving the use of a killing agency concurrently with the application to and distribution through the fabrics under treatment, of a moth repellent, which latter remains in finely divided state, on and in the fabric treated.

Yet another object of the invention is attained in the combined use, requiring only a single stage of treatment, of a liquid hydrocarbon as a killing agent or insecticide, and an inorganic repellent or toxic of water base type, the latter being retained by the cloth or textile as an insectifuge to prevent attack thereof by moth or moth larvae.

Yet another object of the invention is attained in an improved dispersing material, whereby an aqueous solution of an inorganic insectifuge of water-base type may be more evenly dispersed and utilized in a liquid hydrocarbon, than has been possible with dispersing agents heretofore known or used for any similar purpose.

A still further object of the invention is attained in an improved process and mixture for mothproofing woolen garments, which possess a marked economic advantage, due to the use of an extremely low cost toxic or repellent of water base type, and yet which requires materially less water to effect a complete dispersion and distribution of the toxic through the fabric, than in heretofore prevailing processes.

Further objects and advantages of the invention will appear from the following detailed description of certain selected and exemplary practices and materials, all within the scope of the present invention.

Since it is usually quicker and more convenient, particularly in treatment of substantial quantities of fabric such as wool, to effect such treatment by immersion, the process and preferred materials will be described in connection with immersion treatments, although obviously applicable for use in other ways, as by spraying. As a bath for the new treatment, and by preference constituting substantially the major portion of the liquid utilized, there is employed, in substantially known amount, a hydrocarbon preferably having a distinct killing effect on moth and moth larvae, the liquid so utilized being further such that it will evaporate following the treatment so as to leave the cloth or fabric free of this liquid, and any attendant odors, within a reasonable time. The properties noted are

possessed in satisfactory degree by most of the low cost, commercially available liquid hydrocarbons, in which term it is intended to embrace those of petroleum base type, including those produced by distillation or cracking of petroleum, by hydrogenation or polymerization processes, also light hydrocarbons of the nature of petroleum products, such as benzene and casing head gasoline, and still further, those products known in the trade as chlorinated hydrocarbons and including, for example, carbon tetrachloride and trichlorethylene.

In the preparation of the material there may be employed as a toxic or semi-permanent repellent for deposit in and retention by the fabric, any of the fluorides or arsenic salts, the criterion of selection being first, an appreciable or reasonable solubility in water; and secondly, a low cost of the toxic or repellent material. Exhaustive laboratory work based on comparisons of treated fabrics in the presence of moth larvae, with untreated control samples, and taking into account also the quantity of the inorganic toxic or repellent which may be deposited through the use of a limited quantity of water, has indicated magnesium silicofluoride to be considerably superior to the other fluorides and silicofluorides which have come to notice. This preference is further indicated by its appreciably higher solubility than other of the fluorides, particularly in comparison with sodium silicofluoride heretofore utilized to some extent in water solutions for spraying treatments. At usual temperatures of the order of 17.5 degrees C., magnesium silicofluoride may be dissolved in water to the extent of 64.8 percent, while sodium silicofluoride only to the extent of .65 percent. It has been customary in connection with certain practices utilizing the sodium salt, to employ therewith acid solutions of appreciable strength, which obviously will have a detrimental effect on the fibers or textile under treatment. Omitting the acid, it will appear that a given necessarily restricted amount of water utilized as a solvent and carrier for the inorganic toxic, will contain several times as much of the magnesium silicofluoride as of the sodium salt, with proportionate advantages in the retention, by the fabric, of the repellent properties or toxicity against moth.

In view of the noted advantages of magnesium silicofluoride, the steps typifying the use of this as a repellent or toxic, will be described as exemplifying the invention. It is preferred, in order to be assured of standardization of moth-repellent properties and costs, that the repellent, such as magnesium silicofluoride, be employed in quantities definitely proportioned to the dry weight of the fabric to be treated. As a typical example, for each pound of wool to be treated, there is utilized one-fourth ounce of a four to six percent aqueous solution of magnesium silicofluoride. The solution may, if desired, be made somewhat stronger, say up to ten percent. It is also to be noted that the exact quantity of the solution employed per pound of wool, is not critical, and may be varied for example, between limits of one-sixth ounce to one ounce, or if a stronger solution of the fluoride is employed, as little as one-eighth ounce per pound of wool will serve to impart a sufficient amount of toxic repellent to the cloth to prevent, almost indefinitely, any moth damage thereto.

Were the aqueous solution of the fluoride added either directly to the fabric prior to its immersion in the bath aforesaid, or were the solution to be

added directly to the liquid bath, the two liquids, not being inherently miscible, would require extensive and protracted agitation to attain even for a short time, a satisfactory dispersion of the water-toxic solution in the liquid hydrocarbon. Experiments have indicated that, while there are a number of substances which will effect a dispersion to a certain extent, there are wide differences in the manner in which the water solution is absorbed by the fabric, according to the materials employed to effect dispersion. For example, with certain dispersants there is a marked tendency of the cotton portions of clothing, such as men's suits, to absorb the greater part of the aqueous solution with the effect of robbing the wool portions thereof which it is particularly desired to treat against moth attack. It has been determined however that dispersing agents belonging to the class of sulfonated alcohols, and similar materials sometimes referred to as the sulfonated esters of sodium salts, possess the property of causing first, a fine, homogeneous and reasonably enduring dispersion of the water solution in the hydrocarbon bath without requiring an excess of agitation, and secondly, possess distinct advantages in causing absorption of the aqueous solution by the wool desired to be treated, at least equal to the absorption thereof by accompanying cotton or vegetable fibers which obviously require no repellent treatment against moth or the like. While several substances of the general class above referred to are satisfactory for use as dispersing agents, experiments have indicated sulfonated lauryl alcohol as particularly suitable. This material is preferably employed in an amount usually of one-third of one percent of the total weight of liquid, and although the limits are not critical, preferably between one-eighth to three-fourths of one percent of the total weight of liquid, considering all factors, such as cost and dispersing results attained.

It will have appeared from the foregoing that the solution of the toxic-repellent in water in the substantial amounts and proportions stated, having regard for the quantity of wool or fabric under treatment, is then treated with the sulfonated alcohol or ester selected or preferred. The resultant mixture and solution is then added to the liquid hydrocarbon, this mixture being agitated for a short time, a few seconds being usually sufficient. It is immaterial whether the fabric or fabric articles to be treated have previously been immersed in the volatile hydrocarbon, prior to the addition of the prepared aqueous solution including the dispersant, or whether the textiles are immersed following the addition of the solution and dispersant to the hydrocarbon bath. It is preferred for convenience of practice, that the liquids be mixed and the aqueous solution dispersed in the hydrocarbon prior to the immersion treatment of the fabric.

My preference is to agitate the fabric in the liquid as by the use of a washer or drum, or by any other suitable equipment, following which the fabric is removed, the hydrocarbon caused to evaporate therefrom so that the water which will have evaporated by this time or later, will leave an evenly dispersed invisible deposit of the magnesium silicofluoride in intimate union with the fibers throughout the cloth. The moth-repellent properties of the retained salt are such as to render the fabric proof against attack by moths for a substantial period of time, and the toxic-repellent has the further advantage over many of the organic toxics in that it is extremely stable

and unaffected by sunlight as are many of the much more expensive repellants, for example, the quinidine derivatives, rhotenone, and many of the alkaloids and their derivatives.

5 In the practice of the process hereinabove outlined, there results inherently a visual indication of a suitable end point, since, as the aqueous solution containing or including the dispersant is added to the hydrocarbon liquid and agitated, 10 the otherwise clear hydrocarbon becomes opaque or foggy in appearance, due to the finely dispersed particles of the aqueous solution. Continued agitation of the cloth or fabric under treatment in the mixture, causes the foggy appearance or opacity of the liquid to disappear 15 completely, due to the absorption of the aqueous solution by the fabric. This end point is readily observed by change in appearance of the liquid bath, or as observed for example, in a sight glass 20 associated with the agitating apparatus, so that the clothing or fabric may be removed as soon as the hydrocarbon clarifies to a degree approaching normal transparency. When this end point is attained, it may here be noted that only a negligible quantity, say merely a trace, of the aqueous solution remains in the hydrocarbon. This fact 25 results in the advantage of enabling further use of the hydrocarbon for subsequent batches and cycles of treatment with no accumulation in concentration of the aqueous solution, and also enables the use of the subsequent hydrocarbon for any other purpose, such for example as cleaning, or otherwise as may be desired.

It will have appeared that the process described 30 embodies several concurrently practiced steps, viz., the utilization of the hydrocarbon as a medium for killing moth eggs, larvae or insects which may be on the cloth at the time of its treatment. This function of the liquid hydrocarbon is however realized at the same time as its function as a vehicle, carrier or distributing agency for the aqueous solution containing the toxic-repellant. Evaporation of the hydrocarbon and the water, leaves the fabric not only immediately free of all insect life, but proofed 35 against any ravages of moth or the like which might otherwise subsequently take place.

While the invention has been described by making specific and particular reference to exemplary 40 practices and materials employed for the purposes stated, the specification is to be understood not in a limiting, but in a descriptive sense, certain changes in the practice and materials utilized, being possible within the scope of the claims hereunto appended.

I claim as my invention:

1. The process of mothproofing textile fabrics by liquid immersion, which consists in agitating the fabrics in a liquid hydrocarbon bath containing a quantity of an aqueous solution of an in-

organic moth repellant consisting substantially of a relatively soluble fluoride, the solution being dispersed in the liquid hydrocarbon to an extent to produce a visible opacity, proportioning the quantity of the aqueous solution to the weight of the fabric under treatment, and in agitating the fabric in the liquid mixture until substantial clarification of the liquid, as indicating absorption of the aqueous solution by the fabric.

2. The process of mothproofing textile fabrics, 10 which consists in immersion of the fabric in a bath of a liquid hydrocarbon containing a dispersed aqueous solution of magnesium silicofluoride to serve as a moth toxic or repellant in an amount of the order of one-sixth ounce to one 15 ounce of a four to ten percent water solution of the toxic, per pound of dry fabric, and in agitating the fabric under treatment in the liquid mixture for a length of time to cause substantial clarification of the hydrocarbon as indicating substantially complete absorption of the aqueous 20 solution by the fabric.

3. A liquid for the immersion treatment of textile fabrics against moths and like insects, which consists of a quantity of liquid hydrocarbon at 25 least sufficient to saturate the quantity of fabric to be treated, a quantity of magnesium silicofluoride homogeneously dispersed in the hydrocarbon and present therein as an aqueous solution of less than 10% strength, in an amount under one 30 ounce of such solution per pound of fabric to be treated, and a dispersing medium for the magnesium silicofluoride, consisting of a sulfonated alcohol in an amount of the order of 1% of the total weight of liquid.

4. A liquid for the immersion treatment of textile fabrics against damage by moths or like insects, which includes a liquid hydrocarbon in an amount at least sufficient to moisten thoroughly the quantity of fabric to be treated, an aqueous 40 solution of magnesium silicofluoride of a strength of the order of two to ten percent, the magnesium silicofluoride solution being present in the mixture between limits of one-sixth ounce to one ounce, per pound of fabric to be treated, and a 45 dispersing agent in an amount of the order of 1% of the weight of liquid utilized in the treatment.

5. A liquid for the immersion treatment of textile fabrics against damage by moths or like insects, which includes a readily volatile liquid hydrocarbon in an amount at least sufficient to moisten thoroughly the quantity of fabric to be treated, an aqueous solution of magnesium silicofluoride of a strength of the order of four to ten percent, the magnesium silicofluoride solution 50 being dispersed in the hydrocarbon and utilized in the mixture between limits of one-eighth to one-half ounce per pound of fabric to be treated.

AUGUST C. FISCHER. 60